

# UNITED STATES PATENT OFFICE.

HERMAN GABBE, OF BROOKLYN, NEW YORK.

## DRESSING AND DYEING MOLESKINS.

1,384,446.

Specification of Letters Patent. Patented July 12, 1921.

No Drawing.

Application filed April 30, 1919. Serial No. 293,696.

To all whom it may concern:

Be it known that I, HERMAN GABBE, a citizen of the United States, and a resident of the city of New York, borough of Brooklyn, 5 in the county of Kings and State of New York, have invented new and useful Improvements in Dressing and Dyeing Moleskins, of which the following is a full, clear, and exact description.

10 The object of the invention is to provide certain new and useful improvements in the preparation of moleskins for use in fur coats, muffs, scarfs, caps and other fur wearing apparel and whereby the natural color of 15 the moleskin (gray with a bluish tint) is maintained and rendered permanent, and the moleskin is made exceedingly strong and pliable to permit of producing wearing apparel which is durable and highly ornamental and of excellent quality. Another 20 object is to reduce the time required for dressing, dyeing and finishing the moleskin to a minimum thus permitting of manufacturing the skins at a very low cost.

25 With these and other objects in view the invention consists essentially in subjecting the raw moleskin successively to the action of a tanning solution and a dyeing solution, sundry of the ingredients being capable of 30 use in either one of the solutions.

In order to produce the desired result, I proceed in detail as follows: The raw moleskin is soaked in water for about ten hours to soften it and to remove dirt and other extraneous matter. The fur skin is next operated on by a flesher to remove the flesh from the flesh side of the skin and then the skin is placed into a vat containing a tanning solution consisting of alum, salt and 35 soda in about equal proportions. The skin remains in this tanning solution for about two days and is then taken out and its flesh side is oiled and rendered leathery in the usual manner. The skin is next operated on 40 by a flesher to thin down the edges and to remove any flesh that may have been overlooked in the first fleshing operation. The skin is next cleaned of any adhering extraneous matter and is then placed in a vat

containing a dyeing solution consisting, preferably, of—

|                                                         | Parts. |
|---------------------------------------------------------|--------|
| Logwood dye                                             | 50     |
| Sal ammoniac                                            | 25     |
| Sumac                                                   | 25     |
| Bluestone (sulfate of copper)                           | 25     |
| Antimony oxid, known in the trade as<br>needle antimony | 25     |
| Copperas (green vitriol)                                | 50     |

The antimony oxid may be omitted as it is 60 used only to give a darker shade to the fur, if such shade is desired. The sumac and the sal ammoniac instead of being used in the dyeing solution may be used in the tanning solution above referred to. The large proportion of the copperas relative to the bluestone mordant is accounted for by the fact that the bluestone has a coloring strength 65 approximately four times that of the copperas.

70 It is understood that the principal dye (logwood) is of vegetable or organic origin while the mordants (antimony oxid, bluestone and copperas) are of mineral origin, and the sumac is a mordant of organic 75 origin. Nut gall dye about 10 parts is preferably added to the dyeing solution to soften the bluish tint and thus making the fur look richer. It is understood that moleskins from different climates are not alike in 80 the fur and hence the proportions of the ingredients as above given have to be changed correspondingly to produce the desired result.

85 The vegetable dye and the mineral mordants combine to dye the fur to the original color and luster (gray with a bluish tint) of the raw fur and at the same time this color is absolutely fast. The sumac renders the fur exceedingly soft thus causing the hairs to lie down smooth on the skin. The 90 dyeing operation lasts about ten to fifteen hours. After the dyeing is completed the skins are removed from the dye vat and placed in a tumbling barrel containing sawdust, and after this process is completed the skin is 95 ready to be worked into a coat or other fur article.

Having thus described my invention, I

claim as new and desire to secure by Letters Patent:—

1. The herein described composition of matter to be used as a dyeing solution for moleskins, consisting of the following ingredients in about the proportions stated, namely: logwood dye, 50 parts; sal ammoniac, 25 parts; sumac, 25 parts; bluestone, 25 parts; copperas, 50 parts; and antimony oxid, 25 parts.

2. The herein described composition of matter to be used as a dyeing solution for moleskins, consisting of the following ingredients in about the proportions stated, namely: logwood dye, 50 parts; sal ammoniac, 25 parts; sumac, 25 parts; bluestone, 15 25 parts; copperas, 50 parts; and antimony oxid, 25 parts.

HERMAN GABBE.